

## UNITED STATES PATENT OFFICE

ROBERT JAY SHOEMAKER, OF CHICAGO, ILLINOIS, ASSIGNOR TO S. & T. METAL COMPANY, OF CHICAGO, ILLINOIS, A CORPORATION OF ILLINOIS

## BEARING METAL

No Drawing.

Application filed August 2, 1928. Serial No. 297,119.

The invention relates to metallic compositions suitable for bearings, bushings, or other machine elements or parts or articles requiring anti-friction properties or for which a hardened or toughened lead is a proper material.

The principal object of the invention is to provide a lead alloy of this type of suitable hardness, toughness and rigidity for the purposes indicated, which will also have a low coefficient of friction, from which the hardening agents will not drop when the alloy is melted, for example in casting, and which will effectively resist corrosion when exposed to moisture.

A further object is to provide a metallic composition of this type which can be produced conveniently and at low cost. The metallic composition is composed principally of lead to which is added small amounts of other substances, the function of which is to give the lead hardness, toughness, and rigidity. The substances, which may be termed, because of the relatively large quantities used, primary hardeners are tin and calcium. The addition of these substances increases the hardness and toughness of the lead up to a certain point. After a certain amount of calcium and tin have been added to the lead further additions do not result in proportionate increase of hardness. In the case of calcium, particularly, the increase above a certain amount, also gives an undesirable brittleness and makes the alloy unstable when melted or subjected to a moist atmosphere. Apparently lead and tin when melted together in widely varying proportions, perhaps in all proportions, will form a solid solution with no chemical reaction between the substances. This solid solution is harder than lead but the hardening effect is not proportional to the amount of tin therein. In fact the increase of tin above approximately 2.0% does not add to but even, apparently, decreases hardness, so that the use of tin in excessive amount above this percentage is positively a detriment and involves needless expense, tin being more costly than lead. However the detrimental ef-

fect of some excess may be slight, so that it is not possible to definitely fix an upper limit for the tin ingredient, to exclude permissible, through undesirable excesses. The calcium goes into solid solution, apparently, with the lead to the extent of about 0.3% and gives a hardening effect. Above this amount the calcium reacts with the lead to form lead-calcium crystals, when the melt freezes, and these crystals, which are evenly distributed through the mass because they are of substantially the same specific gravity as the lead, give the alloy wearing quality and apparently add somewhat to the hardness. If the calcium is used in excess of 1.0% the metal compound, in its melted state, is viscous and when in the solid state is subject to excessive corrosion in the presence of moisture. I have discovered, further, that if very small amounts of what may be termed secondary hardeners, namely, magnesium, potassium or lithium are incorporated in the lead with the primary hardening agents tin and calcium the hardness and toughness of the compound is increased to quite a surprising extent, without, however, making the alloy either undesirably brittle or subject to dropping or corrosion. These secondary hardeners are to be used in amounts not substantially in excess of 70 their capacities to go into solid solution with the lead. Any excess will react with the lead forming crystals which give rise to inter-crystalline brittleness in the alloy and corrosion along the crystal faces. The practical upper limit for these substances are as given below. Mercury may also be used as a hardening agent, particularly when the secondary hardener is magnesium or potassium, and in any of these compositions the mercury is a desirable element because it decreases the coefficient of friction and gives the surface of the metal, when machined, as in the case of a bearing, a highly polished 75 finish which will remain smooth and shiny for a long time. The alloy also comprises aluminum. The function of the aluminum is to prevent the calcium, magnesium, potassium and lithium from dropping out while 80 85 90 95 100

the alloy is being compounded and also in remelting the ingots for casting for example.

5 The metallic composition consists of the substances above named in proportions, by weight, substantially as follows:

|    |                       |                |                           |
|----|-----------------------|----------------|---------------------------|
| 10 | Tin                   | 0.5% to 2.0%   | Preferable amount 1.0%;   |
|    | Calcium               | 0.3% to 1.0%   | Preferable amount 0.5%;   |
|    | Mercury (optional)    | 0.1% to 0.5%   | Preferable amount 0.25%;  |
|    | Aluminum              | 0.02% to 0.1%  | Preferable amount 0.05%;  |
|    | Magnesium             | 0.05% to 0.1%  | Preferable amount 0.075%; |
|    | Potassium             | 0.02% to 0.06% | Preferable amount 0.04%;  |
|    | Lithium               | 0.02% to 0.06% | Preferable amount 0.04%;  |
|    | Lead to make up 100%. |                | 75                        |

15 The above named alloying substances are melted into the lead, in the manner to be hereinafter described. They all apparently form a solid solution with the lead, to the extent noted, except possibly the aluminum.

20 The amount of aluminum might be increased over that indicated but this would serve no useful purpose and, in fact, amounts larger than those indicated are detrimental in that they make the metal porous.

25 The substances termed secondary hardeners, that is the magnesium, potassium or lithium, appear to be equivalents in some respects. However magnesium is preferred as it appears to give a more stable alloy which can be melted for example in open babbitt kettles without excessive drossing or 30 appreciable loss of hardness.

35 The mercury also has the same effect, as a hardener, whether magnesium or potassium or lithium be used but the increase in hardness which it produces when the last named substances are used is not the same in the case of each of such substances.

40 To illustrate this, a lead alloy compounded in accordance with the preferred proportions, as given in the above table, using magnesium as a secondary hardener will have a hardness of approximately 16° Brinnell if mercury is not used and a hardness of 24° Brinnell when the mercury ingredient is included. An alloy of the same composition 45 except using potassium instead of magnesium will have a hardness of 20° Brinnell without mercury and 26° Brinnell with mercury. Practically it is very difficult to keep more than 0.25% of mercury in the melt because 50 of the tendency of this metal to volatilize at the melting temperatures of the other metals. Its presence in excess of the upper limit indicated is a detriment, for reasons other than expense, because it reduces the melting 55 point of the alloy. Apparently 0.25% of mercury will remain in the alloy regardless of temperature and time of heating.

60 If lithium be substituted for the magnesium or potassium as a secondary hardener the hardness will be approximately 24° Brinnell without mercury and 26° Brinnell with mercury. Thus the mercury, from the point of view of hardness, is more important when the secondary hardener is magnesium 65 or potassium than when it is lithium. The

effect of the mercury in improving the anti-friction qualities is the same in all cases.

70 The secondary hardeners may be used singly as indicated or two of them may be employed or all three. Where two or three of the secondary hardeners are employed they may

be used in amounts which in the aggregate are considerably larger than the upper limit of any of the secondary hardeners used singly. For example, one may add to the lead magnesium up to approximately 0.1 per cent and potassium and also lithium each up to 80 0.06 per cent, and thereby obtain increased hardness, whereas if any single one of the secondary hardeners be used, in an amount corresponding to the aggregate amount in which two or more of the substances are usable the alloy will be unstable and subject to corrosion and drossing. Some increase of the 85 amount of the secondary hardener, magnesium for example, when used alone, over the preferred upper limit as given above is possible although the tendency of the metal to corrosion will be increased somewhat. 90

95 It has been proposed to use lithium, but in relatively large quantities, as a hardener for lead. This substance, however, is very expensive and somewhat difficult to obtain. In the composition above described the lithium is used in such small quantities that the alloy can be manufactured at a very reasonable cost. The same may be said of the magnesium and potassium which are also relatively expensive substances. 100

105 The alloy is compounded preferably in the following manner; the lead is melted to a temperature of approximately 1600° Fahrenheit under a covering of molten calcium chloride. The tin and aluminum are introduced into the lead through the calcium chloride covering, either as metallic tin and aluminum or, which is preferable as a matter of convenience, as a tin-aluminum alloy. The magnesium is next introduced into the 110 lead in the same manner, assuming that this substance is used as a secondary hardener, and thereafter the calcium. The introduction of the calcium into the lead after the other ingredients is a matter of some importance in order to prevent foaming of the calcium chloride covering, which will occur if the calcium is put in first or if all of the beforementioned ingredients are introduced into the lead at one time. The lead is now allowed to cool down to a temperature of about 115 600° to 700° Fahrenheit; or, if desired, the lead with its contents of tin, aluminum, calcium and magnesium may be completely solidified and then remelted to a temperature 120

of not in excess of 700° Fahrenheit. In either case it is desirable to strip off the calcium chloride flux, as soon as this hardens, which will be at the temperature of about 1000° Fahrenheit. If mercury is used, or if the secondary hardener be lithium or potassium these substances, or whichever of them are used, are introduced into the lead while the latter is in a molten state but at the relatively low temperature of 600° to 700° Fahrenheit. At higher temperatures these substances will be volatilized. When lithium or potassium is added it is best to throw some pieces of rosin in the melt and cover the crucible. The rosin burns and drives the air out of the melt and the fumes, if retained in the crucible, prevent the air from coming in contact with the metal. The lithium or potassium should be introduced into the lead while this condition prevails.

One of the important advantages of this form of lead alloy is that it is uniform throughout. There is no segregation as between the upper and lower portions of the ingot. It can be manufactured at low cost. It is very stable, that is it does not readily corrode when exposed to moist atmosphere, nor will the hardening agents dross out to any extent either during the compounding or later if the alloy is melted for casting.

The proportion as between the ingredients, as given above, do not necessarily represent with accuracy the proportions of the substances actually introduced into the molten lead. There will be a certain loss due to oxidation and volatilization. This loss will be greater or less according to the care taken in making the compound. Where the method above described is followed and reasonable precautions are taken the figures in the above table representing the quantities of alloy in substances in the finished composition will very closely represent the quantities introduced into the lead. These figures, however, can only be approximate, and in the present case are arrived at by estimating the losses during compounding and subtracting such estimated losses from the amounts of the ingredients used.

I do not claim herein the method described, as such method is claimed in a copending application, filed October 24, 1930, Serial No. 491,081 as a continuation in part of this application.

I claim:

1. Metallic compound consisting of the following substances in proportions by weight approximately as follows: calcium 0.3% to 1.0%; tin 0.5% to 2.0%; mercury 0.1% to 0.5%; aluminum 0.02% to 0.1%; and metal from the group consisting of magnesium, potassium and lithium 0.02% to 0.22%; together with lead to make up 100%.

2. Metallic compound consisting of the following substances in proportions by

weight substantially as follows: calcium 0.5%; tin 1.0%; mercury 0.25%; aluminum 0.05%; and metal from the group consisting of magnesium, potassium and lithium, 0.075%, 0.04% and 0.04% respectively; together with lead to make up 100%.

3. Metallic compound containing the following substances in proportions by weight approximately as follows: calcium 0.3% to 1.0%; tin 0.5% to 2.0%; aluminum 0.02% to 0.1%; and metals from the group consisting of magnesium, potassium, and lithium 0.02% and 0.22%; together with lead to make up 100%.

4. Metallic compound containing the following substances in proportions by weight substantially as follows: calcium 0.5%; tin 1.0%; aluminum 0.05%; and metal from the group consisting of magnesium, potassium and lithium 0.075%, 0.04% and 0.04% respectively together with lead to make up 100%.

5. Metallic compound consisting of the following substances in proportions by weight approximately as follows: tin 0.5% to 2.0%; calcium 0.3% to 1.0%; mercury 0.1% to 0.5%; magnesium 0.05% to 0.1%; aluminum 0.02% to 0.1%; and lead to make up 100%.

6. Metallic compound consisting of the following substances in proportions by weight approximately as follows: tin 1.0%; calcium 0.5%; mercury 0.25%; magnesium 0.075%; aluminum 0.05%; and lead to make up 100%.

ROBERT JAY SHOEMAKER.

100

105

110

115

120

125

130